

## UNITED STATES PATENT OFFICE

1,990,925

METHOD OF PREPARING A PLATE FOR  
PRINTING PURPOSES

Charles W. Bennett, Douglaston, N. Y., assignor  
to Photo-Cast, Inc., Rochester, N. Y., a cor-  
poration of New York

No Drawing. Original application February 24,  
1933, Serial No. 658,446. Divided and this ap-  
plication July 19, 1933, Serial No. 681,228

16 Claims. (Cl. 41—25)

This invention relates to the preparation of a printing surface by photographic methods, having for its object to provide such a method as will be low in operating costs and more efficient in use than those heretofore proposed.

With these and other objects in view the invention resides in the novel steps and combinations of steps constituting the method as will be disclosed more fully hereinafter and particularly pointed out in the claims.

In order that this invention may be better understood, it is said that there is much need at present for a simplified and an inexpensive method of producing a printing surface, particularly in the reproduction of news and/or copy make-up, to the end that if several steps of the processes now in use can be eliminated, without sacrifice of the resultant printing surface, then much has been attained. This invention therefor is particularly directed to a simplification of preparation of such a printing surface, as well as the novel progressive and intermediate steps which naturally flow from the entire process. In other words, the present novelty lies not only in the production of the finished printing surface, but in the production of a means for photographically developing a sensitized emulsion, as well as in the treatment of the developed emulsion for certain purposes, and also includes the change from one type of emulsion to another during the development.

This invention constitutes a division of that disclosed in my copending application for U. S. Letters Patent filed February 24, 1933 under the Serial No. 658,446 entitled Method of preparing a plate for printing purposes, and also constitutes a continuation in part of that disclosed in my copending application for U. S. Letters Patent filed June 9, 1930 under the Serial No. 460,102 and entitled Method of printing in that this application has for its purpose, the disclosure of a method of preparing a photographic image delineated on a plate and represented by bare and covered portions. While the copending application set forth the production of additional relief in the image on the plate, in this application the additional relief in the image itself is not the primary object, although such may be a secondary occurrence.

The primary object sought herein, is to prepare the same photographic image, laid down in essentially bare and covered parts on the plate, but the covered parts are preferably charged or loaded with a material capable of forming gas when heated. A coating capable of entrapping this gas when evolved, may be added to the image parts

or to the whole surface of the plate (for example, a solution of rubber may be flowed over the entire surface, or such a solution or other sticky films such as rosin in a solvent may be applied selectively, with a roller as in rolling up with ink, to the covered portion representing the image).

Furthermore this gas producing material may be added to the original emulsion of either type (for example, camphor or menthol may be added to the silver type emulsion, or solids, strongly adsorbing gases, may be used as for instance carbon black or clays, as bentonite). In the dichromated emulsion the range of materials is greater and, beside these given above for silver emulsions, there may be added certain salts, such as ammonium carbonate or borate, or organic materials such as chloral hydrate.

These gas forming materials may be added during the developing of a silver image; during the washout process (both types of emulsion) for baring the plate; before, during, or after the final hardening process; and/or placed in or upon the image after hardening. These may be combined and the gas producing material added at more than one point. By way of making the intent more clear, this process cools the plate while the front of the image is heated. Gas is evolved at the heated portions where the cooling is retarded by the image, resulting in increased relief of the casted metal, at such image parts.

It is apparent that such a lag in cooling at the image parts, allows another method of applying the gas forming material namely, to flow over the total surface a gas forming material, or an emulsion or solution of the same (as for instance ammonium carbonate or borate combined with rubber as latex). This surface is then prepared for casting for instance by drying, and casting the hot metal against the above film. Strong cooling at the substantially bare parts prevents a rise in temperature necessary to evolve gas while, at the image parts, the cooling lags and gas is evolved, producing relief sufficient for many cases. This differential liberation of gas is not so generally applicable as the liberation of gas from gas producing material selectively placed in or upon the image parts, either before exposure, or during the process.

According to this process, there is contemplated the provision of a support such as a plate or more especially a paper having thereon an emulsion of the bichromate type with or without an intervening layer of stripping gelatine, the bichromate emulsion having a thickness of as much as seven thousandths of an inch. This

5

10

15

20

25

30

35

40

45

50

55

emulsion is exposed photographically and when the stripping paper is used is then transferred face down to a plate and treated in the usual manner or as hereinafter disclosed to remove the 5 paper back as well as to develop the emulsion to provide bare and covered portions of said plate. If no stripping paper is used then the emulsion is developed immediately after exposure. In this case, and prior to the development, the exposed 10 emulsion may be covered with sticky material as well known, which material may contain the gas producing substance, or said substance may be applied over or under said sticky material. Alternately there may be prepared a silver emulsion 15 over gelatine on a paper support and wherein the thickness of the coating is quite appreciable, such for example as up to five thousandths of an inch for the silver emulsion, the gelatine underlying said emulsion being of any desired 20 thickness and for use in stripping alone. These silver emulsions may be of any suitable and well known formula including the well-known fast silver bromide emulsions of the process type, and containing sufficient silver, of course, so that in 25 the consequent development there will be formed metallic silver. The silver bromide emulsion lends itself admirably to my process.

This sensitized medium is placed in a camera and subjected to light rays admitted through the 30 camera lens to affect the sensitized emulsion in accordance with the object which is being pictured. This sensitized and exposed emulsion is then subjected photographically to development to bring out the latent reproduction or image of 35 said object in black and white. This development of the silver image is properly done at lower temperatures than that of the ordinary and/or heretofore known practice, a practical range being 50-58° F. with considerable lower temperatures giving very good results. During this 40 development the light exposed portions of the emulsion are tanned or rendered insoluble in water, and the resultant developed image strengthened by the partial hardening of the contained gelatine as a result of the tanning. At this point the 45 exposed and developed image now becomes, for all intents and purposes, one of a bichromated type with full light exposure, and in the further consideration of this invention, it will therefore be 50 understood that both the silver and bichromate types of emulsions are equally applicable to the treatment subsequently to be disclosed.

The developer used at this stage of the process is one in which there is used an alkaline carbonate base of such strength as to minimize the 55 swelling of the gelatine, and caustic alkalies to insure penetration, the ratio of carbonate to caustic being adjusted so that the surface development is toned down bearing in mind swelling 60 of the gelatine and penetration of the development. There is also contemplated in this developer a novel medium for reducing the silver of the emulsion to metallic silver which is itself oxidized by the development of the silver salt of the 65 exposed image into a tanning compound, which latter is taken up by the gelatine of the emulsion at the reduced areas only thereof. Also there is preferably provided a restrainer capable 70 of stabilizing the reducer against air oxidation, and an accelerator to restore the normal rate of development without appreciably changing the tendency of the reducer to become air oxidized.

Various chemical elements and compounds 75 may be found suitable for accomplishing this development, as just stated, but from actual prac-

tice it has been found that one which is very efficient and cheap is

|                                                                   | grams |
|-------------------------------------------------------------------|-------|
| Na <sub>2</sub> CO <sub>3</sub> (11% sol.)                        | 1115  |
| NaOH                                                              | 10    |
| KBr                                                               | 6     |
| Na <sub>2</sub> B <sub>4</sub> O <sub>7</sub> ·10H <sub>2</sub> O | 16    |
| CH <sub>3</sub> COCH <sub>3</sub>                                 | 7     |
| K <sub>2</sub> S <sub>2</sub> O <sub>7</sub>                      | 2     |
| C <sub>6</sub> H <sub>4</sub> (OH) <sub>2</sub>                   | 5     |
|                                                                   | 10    |

wherein the sodium carbonate is a water solution and the sodium hydroxide is of 96% purity.

The sodium carbonate is the base having in combination therewith the sodium hydroxide to give penetration in the development, and also in combination with pyrocatechin as the reducing agent. The borax and the potassium bromide form the restrainer, the borax serving to stabilize the pyrocatechin, and the acetone is used as the accelerator, it additionally serving to increase penetration. This acetone also furnishes gas at a later stage of the process since a small quantity thereof is taken up by the gelatine. A small quantity of urea, say up to 3 to 5% of the 15 entire developer volume, may advantageously be used in addition to the foregoing ingredients to assist the penetration of the developer.

This developer has been designed to produce an image with sharp definition and minimum 30 fringe along the developed images thereby producing sharp cut-out. In other words the developer has been made as sharply "contrasty" as possible considering other requirements. This 35 insures a clean washout when the image is subjected to the gelatine-removing washing stage which will be hereinafter disclosed.

This developer can be used at various temperatures, a surprising result being that it has been 40 found that a developer containing a lower concentration of the above ingredients has very successfully worked at a temperature as low as 30° F. and, of course, will likewise work at temperatures thereabove and more in the range of the heretofore known developers. The pyrocatechin 45 in reducing the silver salt of the emulsion of the latent image to metallic silver, concurrently forms a tanning compound acting upon the gelatine of the emulsion at the reduced areas only, to harden the gelatine at said areas, and the 50 hydroxide is found to facilitate the penetration as well as to intensify the tanning action. The developed image may be photographically fixed or not as desired to suit the needs of practice, but I have found it unnecessary to "fix" it. The 55 development is "stopped" by immersion for approximately one minute in a 3% solution of boric acid, then immediately submitted for a short time to an alcohol bath for partial drying.

The developed and partially dried print is then 60 transferred in a well known manner face down upon the surface of a support which may be the surface of a metallic plate or the like, and then the paper backing as well as the stripping gelatine and the whites of the image are washed off 65 leaving the developed and tanned image upon said support. The washing can be done with various chemicals including water, but for extremely satisfactory results an acidified salt solution, such as calcium chloride, has been used. 70 This same washing can be applied to the bichromated type of emulsion as well as to that hereinbefore mentioned.

The chloride is in a solution of substantially 75 5% concentration, and preferably containing 1/2

of 1% of concentrated hydrochloric acid with respect to the volume of the washing solution. A peculiarity of this particular washing solution is that if the chloride is used unacidified, and if a straight hydrochloric acid solution is used, the washing is so materially delayed as to be substantially ineffective; but by acidifying the chloride as above stated, the washing is quickly and efficiently accomplished.

10 As the result of the development, it is highly desirable to keep all portions of the tanned gelatine fixed or immobile with respect to the support to which it is transferred, for should any disturbance of the gelatine occur, there may be a 15 serious defect in the resultant formation of the image, and the printing surface which may be produced therefrom. By the use of this acidified solution of calcium chloride, this result is insured namely, the fixation of the gelatine with 20 respect to the support, in that there is no tendency to loosen the image from the support.

The completely developed and washed image, transferred to the support, is then ready for a further treatment tending to render said image 25 hard and capable of withstanding considerable handling as well as the possible formation of the printing surface in manners including casting of metal against this image. It has been found practical to include in the hardening agent, applied at this stage of the process, a chemical or 30 substance which will be somewhat absorbed by the gelatine so that there will be a quantity thereof in the resultant washed image to produce a gas in the printing surface formation.

35 There is desired a wide latitude in the selection of the gas producing materials since experience has shown that excellent results can be obtained with many. This material may be the hardening solution itself, or it may be added to the washed image before or after the same is hardened by the hardener.

40 Among the gas liberating materials may be found those brought about by (1) reaction, (2) adsorbed gas with slight decomposition, (3) easily decomposable inorganics, (4) volatile or easily decomposable organics. Under the heading of 45 reactions there may be cited chromic acid with oxalic acid as well as chromic acid with hydrogen peroxide, both liberating oxygen, and the former additionally giving off  $\text{CO}_2$ .

50 Among the materials which can be used, covering the second group of adsorbed gas with slight decomposition, there may be listed charcoal, carbon black, fuller's earth, talc, and clays. In addition there are powdered oxides such as 55 litharge, iron oxide, lead dioxide; also powdered metals such as aluminum, and bronze powder; powdered glass such as obtained from a Cottrell precipitator in the stack leading from a furnace burning powdered coal. Also many salts serve admirably for this gas liberating material including Prussian blue; copper, nickel, cadmium, manganese, and calcium oxalates, carbonates, and cyanides; iron carbonate, bismuth sub-carbonate, and bismuth sub-nitrate; Paris green; baking powder, ammonium mercurous chloride; mercury oxides; calcium peroxide; silver-peroxide.

60 Among the easily decomposable inorganics capable of liberating gas will be found sodium perborate, ammonium carbonates, sodium hypochlorite, ammonium borate, ammonium chromates, ammonium oxalate, oxalic acid, and the bicarbonates of alkali metals. On the other hand, the materials which are volatile or easily

decomposable organics and capable of liberating gas, are naphthaline, camphor, acetone, menthol, chloral hydrate, uric acid, milk sugar, pinene (alpha), wintergreen (oil), aniline, aloin, formaldehyde, hydrazine salts such as hydrozine dicarboxylic acid, and organic acids especially the members of the malonic acid series. In addition to the foregoing, water as such, or water of crystallization as in gypsum or calcium sulphate, will also produce evolution of gas upon 10 heat. In any of the foregoing materials it will be understood that they may be added to the hardened image by incorporation in a sticky body which may be rolled on top, or they may be sprinkled over and caused to adhere to the sticky 15 body such as ink which is rolled over the top.

In addition, the finely powdered materials which contain adsorbed gas and when used as gas liberating agents, may be applied over, under, or in the sticky material such as ordinary 20 inks as printing inks or rolling-up inks; rosin in a solvent; varnishes; oils vegetable or animal, straight, bodied by heat, and in combination; aqua resins; galagum in solvent; rubalt (rubber and asphalt); glutrin; rubber in benzol or naphtha, or rubber latex; and collodion in solvent.

It is sometimes desirable to entrap the gas which is liberated from the image so as to accentuate the amount of relief of the image with reference to the support therefor, as well as to 30 insure retention of the gas against loss. Various substances can be used for this purpose, but a solution of dissolved rubber is perhaps the most efficient and may be applied by flowing, or spraying. When using such a rubber solution it will, 35 of course, cover the otherwise bare portions of the metal plate constituting the support for the image as well as the image itself, but this is not detrimental. On the other hand, it is advantageous since it produces a cementitious bond between the metal which may be cast against the 40 image and the support, and the surface of said support, so that additional relief beyond ordinary may be obtained in the resultant cast.

The printing surface is formed preferably by 45 casting type metal or the like against the image and its support. On the other hand, material other than metal such as matrix material, pulp of various forms, etc. may be pressed against the image and its support to receive an impression corresponding to the image, although in the use of the last mentioned materials, no additional relief will result in the ultimate cast. The metal, however, being hot will affect the gas liberating chemical contained in the image, thereby liberating the gas which is then entrapped by the medium or vehicle employed therefor, and the pressure of this gas so liberated will force the metal away from the normal plane of the image so as to add increased relief to the ultimate cast.

The cast can be made in several ways such for 55 example as flowing the molten metal onto the image and its support, or utilizing said support as a wall of a mold, and additionally the metal can be given still further relief by withdrawal of either the supporting plate from the main body portion of the metal, or a withdrawal by vacuum process of a portion of the applied metal while still semi-molten from the supporting plate. It is apparent that the metal can be applied at various pressures other than atmospheric, especially above. In certain instances where desired, the metal plate may be chilled at substantially the time of contact of the molten metal therewith, so as to set or instantaneously 65

solidify said casting metal at the printing surface portion thereof. When the cast is removed, it will be ready to be inked for printing purposes.

It is obvious that those skilled in the art may 5 vary the steps and combinations of steps constituting this method without departing from the spirit of the invention, and therefore it is not desired to be limited to the foregoing except as may be required by the claims.

10 What is claimed is:—

1. The process of producing a printing surface which consists in subjecting a sensitized emulsion on a paper support to photographic exposure; photographically developing said emulsion to obtain 15 an image wherein only the portions acted upon by the light are tanned; transferring the image to a metal plate and washing to remove the paper support as well as to remove the untanned portions of the image down to the plate; 20 treating the transferred and washed image with a hardening agent capable of liberating gas when heated; and forming from the bare portions of the plate a printing surface having a relief greater than the relief of the transferred image, 25 the increase in relief brought about by the liberation of gas from the adsorbed hardening agent.

2. The process of producing a printing surface which consists in subjecting a sensitized emulsion on a paper support to photographic exposure; 30 photographically developing said emulsion to obtain an image wherein only the portions acted upon by the light are tanned; transferring the image to a metal plate and washing with an acidified salt solution to remove the paper support as 35 well as to remove the untanned portions of the image down to the plate leaving the tanned portions unaffected; hardening the transferred and washed image; and forming a printing surface from the bare portions of the plate.

40 3. The process of producing a printing surface which consists in subjecting a sensitized emulsion on a paper support to photographic exposure; photographically developing said emulsion to obtain 45 an image wherein only the portions acted upon by the light are tanned; transferring the image to a metal plate and washing with a solution of approximately 5%  $\text{CaCl}_2$  containing  $\frac{1}{2}$  of one per cent of concentrated  $\text{HCl}$  to remove the paper support as well as to remove the untanned portions of the image down to the plate; 50 hardening the transferred and washed image; and forming a printing surface from the bare portions of the plate.

4. The process of producing a printing surface 55 which consists in subjecting a sensitized emulsion on a paper support to photographic exposure; photographically developing said emulsion to obtain an image wherein only the portions acted upon by the light are tanned; transferring the image to a metal plate and washing to remove the untanned portions of the image down to the plate; 60 treating the transferred and washed image with a hardening agent capable of liberating gas when heated and including formaldehyde; and forming from the bare portions of the plate a printing surface having a relief greater than the relief of the transferred image, the increase in relief brought about by the liberation of gas from 65 the adsorbed formaldehyde.

5. The process of producing a printing surface 70 which consists in subjecting a sensitized emulsion on a paper support to photographic exposure; photographically developing said emulsion to obtain 75 an image wherein only the portions acted

upon by the light are tanned; transferring the image to a metal plate and washing to remove the paper support as well as to remove the untanned portions of the image down to the plate; treating the transferred and washed image with a solution containing chromates of ammonia capable of liberating gas when heated; and forming from the bare portions of the plate a printing surface having a relief greater than the relief of the transferred image, the increase in relief brought 10 about by the liberation of gas from the adsorbed chromates.

6. The process of producing a printing surface which consists in subjecting a sensitized emulsion on a paper support to photographic exposure; 15 photographically developing said emulsion to obtain an image wherein only the portions acted upon by the light are tanned; transferring the image to a metal plate and washing to remove the paper support as well as to remove the untanned 20 portions of the image down to the plate; treating the transferred and washed image with an agent capable of liberating gas when heated; and forming a printing surface from the bare portions of the plate with attendant heat liberating the gas 25 to increase the relief of the printing surface.

7. The process of producing a printing surface which consists in subjecting a sensitized emulsion on a paper support to photographic exposure; 30 photographically developing said emulsion to obtain an image wherein only the portions acted upon by the light are tanned; transferring the image to a metal plate and washing to remove the paper support as well as to remove the untanned portions of the image down to the plate; 35 treating the transferred and washed image with a sticky medium and a material capable of liberating gas when heated; and forming a printing surface from the bare portions of the plate with attendant heat liberating the gas to increase the 40 relief of the printing surface.

8. The process of producing a printing surface which consists in subjecting a sensitized emulsion on a paper support to photographic exposure; 45 photographically developing said emulsion to obtain an image wherein only the portions acted upon by the light are tanned; transferring the image to a metal plate and washing to remove the paper support as well as to remove the untanned portions of the image down to the plate; 50 treating the transferred and washed image with a sticky medium and a salt such as sodium perborate capable of liberating gas when heated; and forming a printing surface from the bare portions of the plate with attendant heat liberating 55 the gas to increase the relief of the printing surface.

9. The process of producing a printing surface which consists in subjecting a sensitized emulsion on a paper support to photographic exposure; 60 photographically developing said emulsion to obtain an image wherein only the portions acted upon by the light are tanned; transferring the image to a metal plate and washing to remove the paper support as well as to remove the untanned portions of the image down to the plate; 65 treating the transferred and washed image with ink and a material capable of liberating gas when heated; and forming a printing surface from the bare portions of the plate with attendant heat liberating the gas to increase the relief of the 70 printing surface.

10. The process of producing a printing surface which consists in subjecting a sensitized emulsion on a paper support to photographic exposure; 75

- photographically developing said emulsion to obtain an image wherein only the portions acted upon by the light are tanned; transferring the image to a metal plate and washing to remove the paper support as well as to remove the untanned portions of the image down to the plate; applying to the covered portions of the plate a material capable of liberating gas together with a vehicle capable of entrapping the gas when 5 liberated; and forming a printing surface from the bare portions of the plate with attendant heat liberating the gas to increase the relief of the printing surface.
11. The process of producing a printing surface 10 which consists in photographing a subject with a plate sensitized with the bichromate type of emulsion having associated therewith a material capable of evolving gas when heated; developing the plate by washing to remove the unexposed 15 emulsion down to the bare plate; and forming a printing surface by molding a substance against the developed and washed plate with attendant heat liberating the gas to increase the amount of relief in the molded substance over the amount 20 of relief in the developed plate.
12. The process of producing a printing surface 25 which consists in photographing a subject on an emulsion of the silver type and having associated therewith a material capable of evolving gas when heated; developing the exposed emulsion and transferring the image to a plate; washing to remove the unexposed emulsion down to the bare plate; and forming a printing surface by molding a substance against the image on the plate with 30 attendant heat liberating the gas to increase the amount of relief in the molded substance over the amount of relief in the transferred image on 35 the plate.
13. The process of producing a printing surface 40 which consists in subjecting a sensitized emulsion on a paper support to photographic exposure; photographically developing said emulsion to obtain an image wherein only the portions acted upon by the light are tanned; transferring the image to a metal plate and washing with an acidified salt solution to remove the paper support as well as to remove the untanned portions of the 45
- image down to the plate; treating the transferred and washed image with a hardening agent capable of liberating gas when heated; and forming from the bare portions of the plate a printing surface having a relief greater than the relief of the transferred image, the increase in relief brought about by the liberation of gas from the adsorbed hardening agent.
14. The process of producing a printing surface 50 which consists in subjecting a sensitized emulsion on a paper support to photographic exposure; photographically developing said emulsion to obtain an image wherein only the portions acted upon by the light are tanned; transferring the image to a metal plate and washing to remove the 55 paper support as well as to remove the untanned portions of the image down to the plate; hardening the transferred and washed image with formaldehyde to incorporate therein a gas producing agent; and forming a printing surface from the 60 bare portions of the plate with attendant heat liberating the gas to increase the relief of the printing surface.
15. The process of producing a printing surface 65 which consists in subjecting a sensitized emulsion on a paper support to photographic exposure; photographically developing said emulsion to obtain an image wherein only the portions acted upon by the light are tanned; transferring the image to a metal plate and washing to remove 70 the paper support as well as to remove the untanned portions of the image down to the plate; treating the transferred and washed image with a sticky medium and a powdered material capable of liberating adsorbed gas when heated; and forming a printing surface from the bare portions of the plate with attendant heat liberating the 75 gas to increase the relief of the printing surface.
16. The process of producing a printing surface 80 which consists in forming upon a plate an image 85 consisting of bare and covered portions of the plate; treating the image with an agent capable of liberating gas when heated; and forming a printing surface from the bare portions of the plate with attendant heat liberating the gas to 90 increase the relief of the printing surface.

CHARLES W. BENNETT.